

March 30, 1954

M. C. HALL

2,673,785

REMOVING CARBON BISULFIDE FROM VISCOSE  
FIBER WITH A LIQUID SEAL VACUUM PUMP  
Filed April 23, 1951



INVENTOR.  
*Myron Charles Hall*  
BY

*Norma E. Rockman*  
ATTORNEY.

## UNITED STATES PATENT OFFICE

2,673,785

## REMOVING CARBON BISULFIDE FROM VISCOSE FIBER WITH A LIQUID SEAL VACUUM PUMP

Myron Charles Hall, Snyder, N. Y., assignor to E. I. du Pont de Nemours &amp; Company, Wilmington, Del., a corporation of Delaware

Application April 23, 1951, Serial No. 222,397

5 Claims. (Cl. 8—137.5)

1

This invention relates to a process for recovering carbon bisulfide from wet acid, gel yarn, filaments, tow or the like produced from viscose by the usual acid-salt bath spinning process.

Numerous methods had been proposed and used for the recovery of carbon bisulfide from wet acid regenerated cellulose yarn and the like made by the viscose process. Many of the prior proposals involve hot-water washing, which is effective but costly in view of the large volume of hot water needed. While it is true that regenerated cellulose yarns can be washed free of not only carbon bisulfide but acid and salt impurities more rapidly with hot water, the time saved is not justified by the additional cost of heating this water. On the other hand, when relatively cool water is used to wash freshly formed regenerated cellulose products, uniform removal of acid and salts is frequently unobtainable in a reasonable time due to the presence of carbon bisulfide which, being insoluble in water and being below its boiling point, is only very slowly dissipated or overcome as a barrier. Furthermore when by using long cycles the removal of acid and salt is completed, the amount of  $CS_2$  remaining is commonly too high to permit processing without elaborate ventilation. If the carbon bisulfide could be economically removed, there would be no serious obstacle to successfully washing the regenerated cellulose structure with cool water to free it from mineral acid, salts, and other by-product impurities.

Generally about 16 to 18 per cent carbon bisulfide remains in the gel yarn or tow as it is collected from the acid spinning bath, based on the dry weight of the regenerated cellulose. Unless this carbon bisulfide is removed down to a value of about four per cent or less based on the dry weight of the cellulose, difficulty will be experienced in uniformly washing the regenerated cellulose product unless the wash water is heated to above the boiling point of the carbon bisulfide. It has been found that a practical solution of this problem is to remove the carbon bisulfide from the acid yarn by a suitable evacuation system hereinafter described, and after this removal of the major portion of carbon bisulfide contained in the yarn, washing with water at a temperature below the boiling point of carbon bisulfide, such as from 30° to 45° C., can be readily and effectively carried out.

It is, therefore, an object of this invention to provide an improved process for purifying and washing regenerated cellulose products produced by the viscose process. Another object of this

2

invention is to provide an improved method for recovering carbon bisulfide from wet acid, gel, regenerated cellulose filaments, yarns, or tows spun from viscose. Still another object of this invention is to provide in combination a suitable carbon bisulfide recovery step followed by an effective washing step for freeing regenerated cellulose filament structures of by-product impurities. These and other objects will be more fully explained in the discussion which follows:

In general the objects of this invention are accomplished by placing the freshly-spun viscose filament product in a sealed chamber and subjecting the same to evacuation by means of a liquid seal pump. The sealing liquid for this pump is maintained at a temperature above the boiling point of the carbon bisulfide to prevent any substantial condensation of the carbon bisulfide thereby.

The liquid seal pump mentioned which is sometimes referred to as a liquid-ring pump, is a ring pump containing an annular body of liquid, formed under the action of centrifugal force, and alternately entering channels formed in the pump casing and in the wings. This type of pump has been used heretofore in connection with carbon bisulfide recovery from viscose rayon products, which process is described in U. S. Patent 2,196,843. In this patent the liquid-seal pump is used in the usual manner, the sealing water being at a relatively low temperature and the carbon bisulfide being condensed thereby. Condensation of the carbon bisulfide in the seal water poses a number of difficult problems: Emulsification of the carbon bisulfide in the water requires the addition of chemical agents to break the emulsion; contact of the condensed carbon bisulfide with metal parts of the pump causes corrosion difficulties; and, probably most important of all, an excessive amount of refrigeration is needed to maintain the seal water at the necessary low temperature to effectively carry out this liquid phase method.

It is generally known that about 80% of the power input to a liquid seal vacuum pump goes into heating the seal water. It would, therefore, seem desirable to operate the pump with seal water at some elevated temperature, which could easily be maintained without excessive cooling of the recirculated seal water. Nevertheless, this idea is directly opposed to the generally accepted and well established practice of using these liquid seal vacuum pumps in that the maximum pumping efficiency can only be realized when relatively cold seal liquor is used. Normally, operating the

pump at relatively low pumping efficiency to produce a minimum absolute pressure no less than about 7 or 6 inches of mercury would indeed seem foolish. In fact, even trying out this system was frowned upon by a number of technical associates of the inventor as being wasteful in time and money; and it might have proved so if some unusual results had not been observed and taken into account in arriving at preferred conditions of operation. For instance, it was found that a relatively poor vacuum was desirable under the conditions obtained, in which the acid yarn or tow was collected as a 33 inch layer in a plurality of compartments in a large rectangular can equipped with a false bottom and was charged into the evacuation chamber at about 38° C. In order to evaporate the carbon bisulfide readily, a relatively high temperature is desirable. It was found that a strong vacuum caused excessive evaporation of water from the rayon tow, with substantial cooling of the yarn mass, and consumed much of the pump capacity with water vapor rather than carbon bisulfide vapor.

Surprising as it may seem, more carbon bisulfide could be evaporated per hour at an absolute pressure of 5-10 inches of mercury, and preferably at a pressure between 5½ and 7 inches of mercury, than could be obtained with the customary high vacuum of about 2 inches of mercury absolute pressure or lower. This was possible not only because the reduced vacuum removed less water vapor but, in view of less water being evaporated, the temperature of the acid regenerated cellulose mass was not appreciably lowered and carbon bisulfide removal was more rapid due to the temperature advantage. At the same time the relatively high temperature of the seal water, which automatically controls the vacuum to cause a high ratio of carbon bisulfide vapor to pass into the pump, caused the carbon bisulfide to stay in the vapor state. This vapor was passed on and separated as an air-carbon bisulfide vapor mixture very readily, permitting easy recovery as will be explained hereinafter. Maintaining the seal water temperature at or around 50° C. may in some cases require only a simple circulating system to utilize heat generated by the pump, excess heat being lost to the atmosphere. However, if use can be made of this low temperature heat, a suitable heat exchanger may be set up and the seal water passed through it.

The single figure of the drawing illustrates by a flow sheet a suitable system for utilizing the present invention.

The wet acid regenerated cellulose product to be freed of carbon bisulfide is placed in vacuum chamber 10. The chamber is connected to liquid seal vacuum pump 11. Water is supplied to the pump from heat exchanger 12 at about 50° C., the flow being adjusted by a solenoid-operated valve 13, to maintain a pressure of 5 to 7 inches of mercury absolute in the cell. Water and carbon bisulfide vapor pass to a separator 14, and separated vapor is passed to a carbon bisulfide recovery system, indicated at 15. Flow of vapor is controlled by a pressure switch 16 and an automatic valve 17.

Water from the separator flows to storage tank 20. The water has been heated by passage 70 through the pump and some cooling occurs during the time it remains in the storage tank. Water is added to the tank at 21 to make up for evaporation occurring in the pump. From the tank the water passes to a centrifugal pump 22 75

and is returned to vacuum pump 11 through heat exchanger 12. The temperature is adjusted to about 50° C. during passage through the heat exchanger by means of control water. The flow of control water is regulated by valve 23. A valve 25 is provided in the line from the vacuum chamber to the vacuum pump for use when the chamber is opened to remove a charge of regenerated cellulose and add a new charge.

To further illustrate the invention, the following specific example is given: Rayon filament tow is collected at the spinning machine in a large rectangular can designed to hold about 600 lbs. of production, figured on an air dry basis. This amounts to about 3,000 lbs. of wet acid tow as collected. The can is divided into three equal compartments, and a false bottom of screen material is located about 2" above the true bottom to allow the escape of CS<sub>2</sub> vapor. The tow is allowed to drop into this can to a total depth of about 33", and evaporation of CS<sub>2</sub>, air and water takes place from only the top and bottom surfaces. The tow, as collected, will contain about 16 to 18% carbon bisulfide, based on the dry weight of the cellulose, or in one can of production there will be about 100 pounds of carbon bisulfide. The can and its contents are charged into vacuum chamber 10, which is then sealed and the liquid seal pump 11, connected therewith is started. Varying the size of charge and varying the vacuum within the chamber by changing the temperature of the seal water gave the following results:

|                                                           | A   | B      | C    | D    |
|-----------------------------------------------------------|-----|--------|------|------|
| Staple Tow Temp. °C.:                                     |     |        |      |      |
| Start.....                                                | 37  | 38     | 38   | 37.5 |
| End.....                                                  | 30  | 31     | 30   | 32.5 |
| Evacuation Time, minutes.....                             | 90  | 90     | 90   | 90   |
| Minimum absolute Pressure, Inches Hg.....                 | 2.0 | 5.7    | 2.4  | 5.5  |
| Weight Sample (in pounds-dry basis).....                  | 600 | 600    | 300  | 277  |
| Percent CS <sub>2</sub> in sample after evacuation.....   | 4.4 | 2.9    | 2.4  | 1.4  |
| Treatment (based on dry sample) Seal Water, Temp. °C..... | 5   | 140-46 | 5    | 50   |
| Percent CS <sub>2</sub> in Wash Effluent:                 |     |        |      |      |
| end 1 hr. wash.....                                       |     |        | .054 | .037 |
| end 2 hr. wash.....                                       |     |        | .037 | .022 |
| end 2½ hr. wash.....                                      |     |        | .022 | .015 |

<sup>1</sup> Recirculated water.

As will be noted from the data above using the preferred conditions of this invention, i. e., seal water at 50° C., over 90% of the carbon bisulfide contained in the acid gel tow charged into the vacuum chamber was removed by the end of one-and-one-half hours. At the end of this time the absolute pressure in the chamber was not below 5½ inches of mercury, which was the minimum pressure obtained.

Following this evacuation treatment the can of rayon tow was removed from the chamber and located in a wash area under suitable sprays, and water at 40° C. and at a pH of 6.75 was showered onto the top of the tow at the rate of about 15 gallons per minute. If free drainage were permitted and the water allowed to run off from underneath the screen as fast as it could, no great depth of water could be maintained in the can, and poor washing efficiency would result. It was therefore found desirable as a result of numerous tests to install a standpipe opening into the bottom chamber of the can and extending above the bottom of the can about 15 inches, or substantially half the depth of the tow contained in the can. This being the only run-off for the water, the discharge rate did not reach the rate of water application to the can until

the can was substantially filled and the surface of the water was above the top layer of tow. At about this position equilibrium was established between the influx and efflux so that this level of wash water was maintained throughout most of the washing cycle. If the porosity of the charge is too little to maintain the water level at the desired point, a suitable control can be installed to maintain the liquid level within the desired limits and without overflowing the can.

The wash cycle is continued for five hours at which time the water spray was shut off and the can of tow removed for further processing. While the carbon bisulfide remaining in the tow after evacuation was in the range of from about 1.5 to 4%, based on the air-dry weight of the tow, at the end of the five hour washing treatment the carbon bisulfide contained in the effluent water was about 0.001%, and the carbon bisulfide concentration in the air above the tank after this purification was of the order of about three parts per million, which is considered very satisfactory.

By this invention it is possible to economically remove carbon bisulfide from wet acid masses of viscose process filaments to the extent of at least 75 or 80% of that originally contained in the acid yarns, and to a sufficiently low value that washing can be effectively carried out with wash water at a temperature substantially below the boiling point of carbon bisulfide. Condensation and final recovery of the carbon bisulfide vapors from the discharge of the water-seal pump is carried out by simple, known methods without need of excessive refrigeration, and because the carbon bisulfide passes through the liquid-seal pump in the vapor state, it has a surprisingly low corrosive effect on the pump parts.

Since many different embodiments of the invention may be made without departing from the spirit and scope thereof, it is to be understood that the invention is not limited by the specific illustrations except to the extent defined in the following claims.

What is claimed is:

1. In a process for purifying freshly spun regenerated cellulose fibers which includes the steps of placing the regenerated cellulose fibers in a closed chamber, then reducing the pressure in the chamber with a liquid seal pump to evaporate carbon bisulfide from the fibers, then removing the regenerated cellulose fibers from the chamber and washing to remove acid and salt, the improvement which comprises maintaining the pump seal water at a temperature around 50° C. to keep the carbon bisulfide in vapor form in the pump discharge and evaporating the carbon bisulfide from the regenerated cellulose fibers at an absolute pressure of 5 to 10 inches of mercury to reduce the carbon bisulfide content of the fibers to less than 4% based on the dry weight of the cellulose, and then washing the regenerated cellulose fibers with wash water at a temperature substantially below the boiling point of carbon bisulfide.

2. A process as defined in claim 1 which includes separating carbon bisulfide vapor and water discharged from the pump, and recirculating the separated water to the pump for reuse as seal water.

3. A process as defined in claim 1 which includes separating liquid water from carbon bisulfide vapor discharged from the pump, condensing the vapor and recovering the carbon bisulfide, then regulating the separated water to a temperature of about 50° C., and recirculating the water to the pump for use as seal water.

4. In a process for purifying regenerated cellulose fibers produced from viscose by the conventional acid-salt bath spinning process using a liquid seal pump to provide reduced pressure for evaporating carbon bisulfide from the freshly spun fibers, the improvement which comprises evaporating carbon bisulfide from the freshly spun regenerated cellulose fibers at an absolute pressure of 5 to 10 inches of mercury while maintaining the temperature of the pump seal water above the boiling point of the carbon bisulfide until the amount of carbon bisulfide remaining in the fibers is less than 4 percent based on the dry weight of the cellulose, and then washing the fibers with wash water at a temperature substantially below the boiling point of carbon bisulfide until substantially all of the acid, salt and remaining carbon bisulfide are removed.

5. In a process for purifying freshly spun regenerated cellulose fibers which includes the steps of placing regenerated cellulose fibers in a closed chamber, then reducing the pressure in the chamber with a liquid seal pump to evaporate carbon bisulfide from the fibers, then removing the regenerated cellulose fibers from the chamber and washing to remove acid and salt, the improvement which comprises maintaining the pump seal water at a temperature around 50° C. to keep the carbon bisulfide in vapor form in the pump discharge and evaporating the carbon bisulfide from the regenerated cellulose fibers at an absolute pressure of between 5½ and 7 inches of mercury until the carbon bisulfide remaining amounts to 1.5% to 4% based on the dry weight of the cellulose, and then washing the regenerated cellulose fibers with wash water at 30° C. to 45° C. until substantially all of the acid, salt and remaining carbon bisulfide are removed.

MYRON CHARLES HALL.

References Cited in the file of this patent  
UNITED STATES PATENTS

| Number     | Name                 | Date          |
|------------|----------------------|---------------|
| Re. 20,079 | Moritz et al. -----  | Aug. 25, 1936 |
| 1,579,711  | Kampf -----          | Apr. 6, 1926  |
| 1,907,101  | Funcke et al. -----  | May 2, 1933   |
| 2,035,981  | Richter -----        | Mar. 11, 1936 |
| 2,133,244  | Baumert et al. ----- | Oct. 11, 1938 |
| 2,196,843  | Van Deinse -----     | Apr. 9, 1940  |